

## UNITED STATES PATENT OFFICE

VAN M. DARSEY, OF DETROIT, MICHIGAN, ASSIGNOR TO PARKER RUST-PROOF COMPANY, OF DETROIT, MICHIGAN, A CORPORATION OF MICHIGAN

## COATING METAL

No Drawing.

Application filed May 13, 1929. Serial No. 362,873.

This invention relates to coating metal, and more particularly to treatment in connection with coating iron or steel with phosphates.

It has been a common practice for some years to boil iron or steel articles in a dilute solution of phosphoric acid, or phosphates, and thereby coat the surface with a comparatively insoluble coating of phosphates. Recently it has been discovered that the addition of a compound of copper to the solution greatly increases the rapidity with which the phosphate coating is deposited, but at the same time metallic copper is deposited, interspersed through the phosphate coating.

The coating with copper interspersed therethrough is suitable to form a base for paint, enamel or the like, but does not of itself form a satisfactory rustproofing. Probably the rusting of the iron is accelerated by the electric action due to the copper adjacent thereto.

It is one purpose of this invention to treat such a phosphate and copper coating so as to greatly increase its resistance to rusting.

Articles coated with a phosphate and copper coating dipped in a hot solution of potassium chromate for a brief period resist rusting about as well as similar articles coated with the phosphate coating without the copper, and the phosphate and copper treatment and subsequent treatment with the chromate solution requires much less time than the formation of the coating of phosphates alone. The chromate solution has no visible or chemically ascertainable effect upon either the phosphate coating or the copper, but probably it affects the electrical action of the copper. At any rate, it very markedly retards the rusting of the articles treated.

The preferred strength of the chromate solution is from 1 to 5 grams per liter of water, but the strength of the solution may be even more widely varied without injurious results. The strength of the solution does

not have any marked effect on the result. A cold solution has a similar effect but acts much more slowly than the hot solution.

Potassium dichromate may be used also, and other soluble chromates and dichromates may be employed, if preferred. Chromic acid ( $\text{CrO}_3$ ) may be employed instead of the chromates, but care must be taken not to use too strong a solution. A solution of two or three grams to a liter of water works fairly well, but over three grams to the liter perceptibly injures the phosphate coating. For this reason a chromate solution is preferred to a chromic acid solution.

It is sometimes desirable to reduce the amount of copper deposited in the coating. Dipping the articles in a hot chromate solution before placing them in the phosphate and copper bath retards the deposition of copper while at the same time it reduces the time in which the reaction of the bath with the articles is completed. Preliminary dipping in a chromic acid solution likewise retards the deposition of copper, but it retards the formation of the phosphate coating, instead of accelerating it, as the chromate solution does.

When a soluble salt of lead is added to a phosphate coating bath, lead is not deposited to any appreciable extent in the absence of some other added material; but when a little soluble salt of copper is added, the lead is deposited very rapidly, and forms with phosphates a somewhat soft and smudgy coating. Treatment of the articles in a chromate solution before subjecting them to the phosphate-lead-copper bath retards the deposition of the lead and improves the coating. Treatment of the thus coated articles with a chromate or chromic acid solution improves its rust-resisting qualities. The chromic acid solution for the coating containing lead is more desirable than with a coating containing copper, but free from lead, as lead forms a substantially insoluble chromate.

While the phosphate coatings mentioned above as being benefited by treatment with a chromate solution were only those containing copper or lead, it will be understood that phosphate coatings containing other metals having a different electric potential from iron may be rendered more rust-resistant by treatment in a solution containing a soluble chromate or chromic acid, and that treatment of iron or steel with a solution containing the chromic acid radical before treatment in a phosphate bath retards the deposition on the iron of other metals which are less basic than iron and which are dissolved in the phosphate bath.

From the above, the nature of the invention and the manner of its use will be apparent to those skilled in the art.

What is claimed is:

1. The method which consists in treating an article having a surface of iron or steel bearing a phosphate coating containing a metal having a potential different from that of iron or steel, with a solution of a material containing the chromic acid radical.

2. The method which consists in treating an article having a surface of iron or steel bearing a phosphate coating containing a metal having a potential different from that of the iron or steel, with a solution of a salt of chromic acid.

3. The method which consists in treating an article having a surface of iron or steel bearing a phosphate coating containing a metal with a potential different from that of the iron or steel of said surface, with a hot dilute solution of a material containing the chromic acid radical.

4. The method which consists in treating an article having a surface of iron or steel bearing a phosphate coating containing a metal with a potential different from that of the iron or steel of said surface, with a hot solution of a salt of chromic acid.

5. The method which consists in treating an article having a surface of iron or steel bearing a phosphate coating containing a metal less basic than iron, with a solution of a material containing the chromic acid radical.

6. The method which consists in treating an article having a surface of iron or steel bearing a phosphate coating containing copper, with a solution of a material containing the chromic acid radical.

7. The method which consists in treating an article having a surface of iron or steel bearing a phosphate coating containing copper, with a hot solution of an alkali salt of chromic acid.

8. The method which consists in treating an article having a surface of iron or steel bearing a phosphate coating containing copper, with a hot dilute solution of potassium chromate.

9. The method which consists in treating an article having a surface of iron or steel bearing a phosphate coating containing a metal with a potential different from that of the iron or steel of said surface, with a hot dilute solution of an alkali salt of chromic acid.

10. The method which consists in treating with a solution containing the chromic acid radical an article having a surface of iron or steel, immersing the treated article in a dilute phosphate solution containing in solution a metal less basic than iron and thereby coating said surface with a phosphate coating containing said metal less basic than iron, and treating the coated surface with a solution containing the chromic acid radical.

11. The method which consists in treating with a solution of a salt of chromic acid an article having a surface of iron or steel, immersing the treated article in a dilute phosphate solution containing in solution a metal less basic than iron and thereby coating said surface with a phosphate coating containing said metal less basic than iron, and treating the coated surface with a solution of a salt of chromic acid.

12. The method which consists in treating with a solution of a salt of chromic acid an article having a surface of iron or steel, immersing the article in a hot dilute phosphate solution containing a soluble compound of copper, until a phosphate and copper coating is formed on said surface, and treating the coated surface with a solution of a salt of chromic acid.

13. The method which consists in treating an article having a surface of iron or steel with a hot dilute solution of alkali chromate, immersing the treated article in a hot dilute phosphate solution containing copper in solution, until said surface is coated with copper and phosphate, and treating the coated surface with a hot dilute solution of alkali chromate.

14. The method which consists in treating with a solution containing the chromic acid radical an article having a surface of iron or steel, and immersing the treated article in a dilute phosphate solution containing in solution a metal less basic than iron and thereby coating said surface with a phosphate coating containing said metal less basic than iron.

15. The method which consists in treating with a hot dilute solution of alkali chromate an article having a surface of iron or steel and immersing the treated article in a hot dilute phosphate solution containing a soluble compound of a metal less basic than iron, and thereby providing said surface with a phosphate coating containing said metal less basic than iron.

16. The method which consists in treating an article having a surface of iron or steel

with a hot dilute solution of an alkali salt of chromic acid, and immersing the treated article in a hot dilute phosphate solution comprising copper phosphate in such proportions with phosphates of metals which form both soluble and substantially insoluble phosphates that a coating is formed on said surface containing metallic copper and substantially insoluble phosphates of other metals.

5 <sup>10</sup> In testimony whereof I have hereunto signed my name to this specification.

VAN M. DARSEY.

15

20

25

30

35

40

45

50

55

60

65